

R. E. OTTMAN.

INSULATING MATERIAL AND METHOD OF MAKING SAME.

APPLICATION FILED DEC. 10, 1917.

1,418,730.

Patented June 6, 1922.



INVENTOR:  
Robert E. Ottman  
by J. G. Roberts Atty

# UNITED STATES PATENT OFFICE.

ROBERT E. OTTMAN, OF EAST ORANGE, NEW JERSEY, ASSIGNOR TO WESTERN ELECTRIC COMPANY, INCORPORATED, OF NEW YORK, N. Y., A CORPORATION OF NEW YORK.

## INSULATING MATERIAL AND METHOD OF MAKING SAME.

1,418,730.

Specification of Letters Patent. Patented June 6, 1922.

Application filed December 10, 1917. Serial No. 206,453.

To all whom it may concern:

Be it known that I, ROBERT E. OTTMAN, a citizen of the United States, residing at East Orange, in the county of Essex, State 5 of New Jersey, have invented certain new and useful Improvements in Insulating Materials and Methods of Making Same, of which the following is a full, clear, concise, and exact description.

10 This invention relates particularly to a material for use between the rows of dry cells in dry cell battery cabinets, but may also be availed of wherever similar insulating problems are presented.

15 In dry cell battery cabinets the cells are often so connected that a difference of potential as high as 100 volts may exist between two cells in adjacent rows. It is, therefore, desirable that adjacent rows of cells be separated by some insulating material in addition to the pasteboard cartons containing 20 individual cells. As a result of exposure to electrolyte leaking from cells whose zinc casings have become perforated after long or 25 heavy service, this insulating material, if it absorbs moisture or is chemically attacked by the constituents of the electrolyte, loses its insulating efficiency and permits short-circuits which result in a heavy flow of current and possibly in ignition of the cartons or separators. There is also a fire risk from 30 cells which, on account of long use, have a high internal resistance, since, if a short circuit develops either between cells or in 35 the wiring, the resulting heavy flow of current may heat up the carbon in these old cells to such an extent as to ignite either the cartons or the separators and even the cells themselves.

40 It is, therefore, an object of my invention to provide an insulating material adapted for use between the cells of dry cell batteries, which is substantially nonignitable and therefore fire-proof and which retains its insulating efficiency when exposed to the action of 45 the contents of the cells.

The single figure of the drawing shows, in perspective, an embodiment of my invention comprising a sheet of electrically non-conducting fabric which may be stiff paper or thin flexible cardboard, and which has

been impregnated with suitable ignition preventives. The process of impregnation preferably consists of immersing sheets or strips of the paper, cardboard or other fabric in a 55 solution containing the ignition preventives, a suitable solution comprising borax and ammonium phosphate in the proportions of one pound of borax (commercial grade) and three pounds of ammonium phosphate (commercial grade) to twenty-five pints of water. The paper or cardboard is kept in the solution until it is completely impregnated therewith, after which it is thoroughly dried.

Each side of the dried fabric is coated 65 with a moisture-proof paint which may suitably consist of 40% (by weight) of linseed oil and 60% (by weight) of a mixture of—

|                   |     |    |
|-------------------|-----|----|
| Zinc oxide        | 54% | 70 |
| Calcium carbonate | 45% |    |
| Lamp black        | 1%  |    |

This composition is not only a moisture resistant and unaffected chemically by sal ammoniac, zinc-chloride or other common 75 constituents of dry cell electrolytes, but as it is electrically non-conductive, it adds considerably to the insulating efficiency of the fabric and counteracts any contrary effect due to the presence of the fireproofing salts. 80 Each side of the fabric preferably receives a double coating of this compound.

The finished material is easily cut into desired shapes, and being tough and resili- 85 ent, readily adapts itself to the spaces between battery cells or the like. It does not absorb moisture nor is it chemically attacked by the constituents of dry cell electrolytes; it can be ignited only with difficulty, and if ignited does not continue to burn; and it is 90 a non-conductor of electricity. It is, therefore, particularly adapted for use as a separator between the cells of dry cell batteries and for similar purposes.

What is claimed is:

1. The method of forming an electrically insulating material which consists in impregnating a non-conductive fabric with a solution of borax and ammonium phosphate, drying the impregnated fabric, and coating 100 said fabric with a mixture of calcium carbonate, zinc oxide and linseed oil.

2. An electrical insulating material comprising a sheet of fabric impregnated with borax and ammonium phosphate, and having a waterproof coating.
- 5 3. An electrical insulating material comprising a sheet of fabric impregnated with borax and ammonium phosphate, and hav-

ing a coating comprising calcium carbonate, zinc oxide and linseed oil.

In witness whereof, I hereunto subscribe to my name this 5th day of December A. D., 1917.

ROBERT E. OTTMAN.